

## 1

2,833,670

## AFTER-TREATMENT OF TEXTILE FABRIC HAVING CURED FORMALDEHYDE LIBERATING RESINS AND ARTICLE FORMED THEREBY

Philip B. Roth, Somerville, N. J., assignor to American Cyanamid Company, New York, N. Y., a corporation of Maine

No Drawing. Application June 13, 1956  
Serial No. 591,013

10 Claims. (Cl. 117—62)

The present invention relates to the after-treatment of textile fabrics having a cured formaldehyde liberating resin or resin mixture thereon with a formaldehyde acceptor and to the fabrics so treated.

In recent years, the use of durable finishes for textiles has been of considerable importance in the textile industry. These finishes have imparted various properties, as for example, a firm resilient hand, wrinkle resistance, shrinkage control, water repellency, flame resistance, spot resistance and the like.

Many of these finishes are obtained by using thermosetting resins wherein formaldehyde is an essential component of the resins and resin mixtures. Thus, urea-formaldehydes, melamine-formaldehydes, urea-thiourea mixed resins and their sulfonated derivatives and/or their alkylated derivatives are examples of important resins in this field.

In many instances, the nature of the finish depends to some extent on the amount of the thermosetting resin employed. A desirable hand for lightweight woven synthetic fabrics may be obtained by using from  $\frac{1}{2}$  to 2% of a urea-formaldehyde resin. Increasing the amount of resin solids to from between 5 and 15% gives a stiffer hand and improves wrinkle resistance and shrinkage control of the cellulosic fabrics. Modifying the urea-formaldehyde by incorporating thiourea-formaldehyde and partially alkylating both resins improves the flame resistance and increases the stiffness of textile materials, such as nylon. In the latter instance, concentrations of the order of 30 to 80% resin solids based on the weight of the fabric are frequently employed.

Regardless of which resin is used, fabrics which have been treated therewith tend to liberate formaldehyde upon storage. This is a problem of considerable concern in the industry in that fabrics so treated and having such a limitation are difficult to handle and, in addition, result in health hazards, both of which are undesirable.

The cause of formaldehyde liberation may be due, at least in part, to the acid pH of the treated fabric. Attacking the problem from this aspect, alkaline agents have been incorporated into pad baths in order to reduce the amount of available free formaldehyde therein and also to reduce the amount of formaldehyde which may be liberated upon storage. If formaldehyde acceptors are added in the pad bath, the amount of formaldehyde which is liberated on storage is somewhat reduced but the rate of cure of the fabric is considerably retarded and makes it extremely difficult, particularly where the fabric is nylon, to obtain a suitable stiff hand without destroying the saleability of the fabric. After-treating of cured formaldehyde liberating resins with various alkaline agents such as ammonium hydroxide, sodium carbonate and other materials, has also been tried. When these materials are employed in practical amounts, the amount of

## 2

liberated formaldehyde is reduced insufficiently to render the process of commercial importance.

Accordingly, it is an object of the present invention to provide a process for preventing the liberation of formaldehyde from a fabric having a cured formaldehyde liberating resin thereon or reducing the amount so liberated to an acceptable commercial level.

It is a further object to provide such a process which is adaptable to conventional mill equipment and which therefore may be practiced easily and relatively inexpensively with existing equipment.

A particular object of the present invention relates to a process for reducing the amount of formaldehyde liberated from a fabric having a cured formaldehyde liberating resin thereon wherein the resin is of the type such as mixed urea-thiourea-formaldehyde type, which may be partially alkylated or partially polymerized and which may further be bisulfite modified. These resins are normally used in rather high solids content (30-80% based on the weight of the fabric) in that one of their principal functions is to impart a springy resilient hand to nylon fabrics without increasing their combustibility.

The resin-treated fabric having a cured formaldehyde liberating resin thereon which will yield amounts of free formaldehyde in excess of 0.3% based on the weight of the fabric when stored for 20 hours at 100° F. and at a 100% relative humidity have been determined to be commercially undesirable. Accordingly, resin-treated fabrics having cured formaldehyde liberating resins thereon which liberate 0.3% and less based on the weight of the fabric of formaldehyde when stored under the above conditions are for the most part acceptable in the trade.

A simple test has been devised to determine the amount 35 of formaldehyde liberated by a fabric treated with a formaldehyde liberating resin. In principle, a piece of a fabric treated with a formaldehyde liberating cured resin is weighed and placed in a bottle, as for example a 4-ounce bottle in the presence of an excess of water, as 40 for example 50 cc. The fabric is suspended so as not to be immersed in the water and the jar is tightly capped, excluding all air. The bottle is stored at 100° F. for 20 hours, the fabric is removed, and the bottle is shaken to absorb all the formaldehyde liberated by the fabric.

45 Thereafter, the formaldehyde is analyzed by forming a color compound with chromotropic acid solution and the percent of formaldehyde is estimated by the depth of the color which may be determined either spectrophotometrically or by comparing with standards of known concentration. This percent is then correlated to the weight of the fabric. The water is present in the container in excess of the amount necessary to saturate the atmosphere or air space in the closed bottle. This is to assure a 50 relative humidity of 100%. If a treated fabric yields 55 formaldehyde in amounts in excess of 0.3%, it is unacceptable for most commercial usage.

According to the present invention, a process is provided for reducing the amount of formaldehyde liberated from a fabric having a cured formaldehyde liberating resin thereon, which resin is capable of liberating formaldehyde in amounts in excess of 0.3% based on the weight of the fabric when stored for 20 hours at 100° F. and at 100% relative humidity. The process comprises after-treating such a resin-treated fabric with an amount 60 of a formaldehyde acceptor, sufficient to reduce the amount of formaldehyde liberated when a fabric so treated is stored for 20 hours at 100° F. and at 100% relative humidity to 0.3% and less formaldehyde based on

the weight of the fabric. Thereafter, the fabric is dried. By "formaldehyde acceptor," as the term is used herein, it is meant any compound which is capable of reacting with formaldehyde to prevent volatilization of formaldehyde from formaldehyde liberating resins and resin mixtures which have been cured on textile fabrics. Preferably, the term is intended to include compounds which so react at room temperature or at temperatures either below or slightly above and which will not discolor the fabric which they are used to treat. The formaldehyde acceptors are preferably water-soluble amino and amido compounds, although other formaldehyde acceptors, either of these classes or of other classes which are not fully water soluble at room temperature or at elevated temperatures, but are soluble or may be rendered sufficiently soluble by the use of organic solvents such as acetone, alcohols and the like, may be employed.

Suitable formaldehyde acceptors within the meaning of the present invention include urea, dicyandiamide, ethylene urea, propylene urea, methylene urea, oxamide, propio-1,3-diamide, succinamide, propionamide, melamine; certain guanamines; polyamines such as ethylene diamine and propylene diamine; primary amines such as methyl amine and ethyl amine; alcohol amines such as ethanol amine and propanol amine; guanidine and guanidine salts; mono and poly urethanes; and 5-methyl hydantoin, and the like. These nitrogenous compounds capable of reacting with formaldehyde to form condensation products or their functional equivalents may be used either singly or in combination.

These acceptors may be applied to the fabric by spraying a solution thereof or by passing the fabric to be treated through a solution and then removing the excess by passage through squeeze rolls. Other suitable means may also be employed. As noted above, the aqueous spray or pad bath solution may be aqueous, solvent or an aqueous-solvent mixed solution that contains sufficient organic solvent to assist in solubilizing a sufficient amount of the acceptor to produce an effective solution.

The temperature of the spray or padding solution may be room temperature, i. e. about 25° C. This is particularly desirable if the formaldehyde acceptors require the use of an organic solvent to achieve the desired degree of solubility, in that volatilization and in some cases the undesirable generation of odors may be overcome. On the other hand, if the solubility of the formaldehyde acceptor is increased by raising the temperature of the solution slightly, there is no objection in employing an elevated temperature. High temperatures near the boiling point of the spray or padding solution should be avoided, to avoid endangering the durable nature of the resin finish.

After the application of the formaldehyde acceptor, the after-treated fabric may be dried at room temperature or if necessary at somewhat higher temperatures, being careful not to scorch the fabric. Preferably, the after-treated fabric is dried at between room temperature and 50° C.

While, generally speaking, the process of the present invention is applicable to any resin-treated fabrics wherein the cured resin is capable of liberating formaldehyde

in excess of the 0.3% based on the weight of the fabric as defined above, it is particularly applicable to those resin-treated fabrics wherein the percent of liberated formaldehyde is in excess of 1% by the same test. Even more specifically, the process of the present invention is principally directed at cured resin-treated fabrics which, when subjected to the same test, liberate amounts of formaldehyde between 1 and 3% based on the weight of the fabric.

I have found that when resin-treated fabrics liberate formaldehyde in the amounts of between 1 and 3% that the process of the present invention is particularly effective when the formaldehyde acceptor is applied in amounts of between 5% and 10% based on the weight of the fabric. Obviously, in some instances, slightly lower and slightly higher percentages are required or may be required to achieve the desired degree of after-treatment effectiveness. However, for the most part, treatment with formaldehyde acceptors within this range produce eminently satisfactory results.

If the amount of formaldehyde liberated is between 0.3 and 1%, smaller amounts (sufficient to reduce the liberated formaldehyde to 0.3% or less) of formaldehyde acceptor of the order of about 2% based on the weight of the fabric are in most instances effective. Likewise, if a resin-treated fabric had a cured formaldehyde liberating resin thereon which would liberate formaldehyde in excess of 3% based on the weight of the fabric, amounts up to about 15% of acceptor based on the weight of the fabric may be employed.

In order that the present invention may be more fully understood, the following examples are given primarily by way of illustration. No specific details therein should be construed as limitations except as they appear in the appended claims. All parts and percentages are by weight unless otherwise designated.

#### Example 1

Eighty parts by weight of a bisulfite-modified partially methylated urea-thiourea-formaldehyde resin product, 0.52 part of ammonium chloride, and 19.40 parts of water sufficient to yield a total of 100 parts are made up into a padding solution containing 64% solids. Through this padding solution, nylon Rochelle netting was passed and the excess of the pad bath solution was removed by squeeze rollers so that the fabric retained 100% of its weight of the treated solution. The treated fabric was then heated for 60 seconds at 310° F. after which it was cooled to room temperature and sprayed with a 5% solution of urea. The fabric was then dried at room temperature.

#### Example 2

Example 1 was repeated except that in the afore-treatment the fabric was treated with 10% of urea based on its weight. Thereafter, the fabric was dried at room temperature.

#### Example 3

The procedure of Example 1 was followed except that there was no after-treatment with urea. This example was used as the control in the data recorded in the chart set forth hereinbelow.

| Treatment                                              | After 20 hours' storage at 100° F. and 100% RH—percent formaldehyde liberated | Odor        | Hand | Color | Fire Retardancy |
|--------------------------------------------------------|-------------------------------------------------------------------------------|-------------|------|-------|-----------------|
| Example No. 3 (Control).....                           | 1.8                                                                           | Sl. HCHO    | Std. | Std.  | OK              |
| Example No. 1 sprayed with 5% urea <sup>1</sup> .....  | 0.8                                                                           | V. sl. HCHO | Std. | Std.  | OK              |
| Example No. 2 sprayed with 10% urea <sup>1</sup> ..... | None                                                                          |             | Std. | Std.  | OK              |

<sup>1</sup> Adds 5 and 10% urea based on weight of cloth.

It will thus be observed that the omission of the use of a formaldehyde acceptor as an after-treatment resulted in 6 times as much formaldehyde being liberated as when the after-treatment with 5% of urea based on the weight of the fabric was employed. In addition, it will be noted that when a 10% urea was employed, no odor of formaldehyde developed whatsoever under the above test conditions nor was there any detrimental effect on the hand, color or fire retardancy of the nylon fabric.

*Example 4*

Nylon Rochelle netting was treated as in Example 1 except that a 5% solution of succinamide in acetone was used in place of the aqueous urea solution. After this treatment the fabric liberated less than 0.3% formaldehyde.

The process of the present invention is particularly adaptable to resin-treated fabrics having cured formaldehyde liberating resins which liberate formaldehyde in amounts on the order of from 1 to 3% when subject to test conditions set forth above. Resins which liberate formaldehyde in these amounts under the test conditions are, for the most part, resins which are applied in rather large quantities, as for example, of the order of 30 to 80% or more based on the weight of the textile fabric. In particular, the resins adapted to impart flame resistance to nylon fabrics may be considered to be within this class. Here, the resins are added on in rather large amounts in order to impart the desired degree of resiliency and stiffness to the particular fabrics.

A resin composition of this type, when applied to nylon netting to give about a 60 to 80% solids add-on, imparts a springy hand to the fabric and also retains the burning characteristics of the untreated nylon. However, on storage, formaldehyde is liberated and the obnoxious odor which results is undesirable.

As another example of a resin which liberates formaldehyde and which is added to nylon fabric to impart a springy hand and which is added on in relatively large quantities are partially alkylated thiourea-formaldehyde resinous compositions. These resinous compositions which contain on the order of about 50% thiourea can be blended with partially polymerized urea-formaldehydes, methylated methylol melamines or dimethylol thiourea to yield mixtures containing on the order of about 18% thiourea. An important disadvantage of them is the fact that they liberate formaldehyde when stored.

An additional example of such resins and the resin employed in the treatment of nylon in Examples 1 to 4 are the partially alkylated, partially polymerized urea-thiourea resin which is bisulfite modified.

These resins, as well as any resin which would liberate formaldehyde in amounts in excess of 0.3% based on the weight of the fabric in accordance with the test above-defined may be applied to the fabric by any one of a large number of conventional processes well-known in the art. For example, a pad bath may be prepared containing the correct amount of solids to produce the desired finish and a catalyst such as an ammonium halide, an alkali metal salt, amine hydrochlorides or organic acids such as oxalic or tartaric may be added to the bath. Water may be then added to give the correct concentration of solids and the fabric padded therethrough, the excess of the pad bath solution being removed by squeezing, centrifuging, or other means. Thereafter, the fabric is dried and the resin cured, as for example, for 5 minutes at 250° F. to 5 seconds at 450° F. and preferably for from 1 to 3 minutes at from 360° F. to 290° F., depending upon the nature of the fabric and the cure desired.

I claim:

1. A process for reducing the amount of formaldehyde liberated from a fabric having a cured formaldehyde liberating resin thereon, said cured resin being capable of liberating formaldehyde in amounts in excess of 0.3% based on the weight of the fabric when stored for 20

hours at 100° F. and at 100% relative humidity, which comprises after-treating said resin-treated fabric with an amount of a formaldehyde acceptor, said formaldehyde acceptor being a nitrogenous compound capable of reacting with formaldehyde to form a condensation product, said amount being sufficient to reduce the amount of formaldehyde liberated when fabric so treated is stored for 20 hours at 100° F. and 100% relative humidity to 0.3% and less based on the weight of the fabric, and thereafter drying the fabric.

2. A process for reducing the amount of formaldehyde liberated from a fabric having a cured formaldehyde liberating resin thereon, said cured resin being capable of liberating formaldehyde in amounts in excess of 0.3% based on the weight of the fabric when stored for 20 hours at 100° F. and at 100% relative humidity, which comprises after-treating said resin fabric with an amount of an amide, formaldehyde acceptor, said amide acceptor being applied in an amount sufficient to reduce the amount of formaldehyde liberated when fabric so treated is stored for 20 hours at 100° F. and 100% relative humidity to 0.3% and less based on the weight of the fabric, and thereafter drying the fabric.

3. A process for reducing the amount of formaldehyde liberated from a fabric having a cured formaldehyde liberating resin thereon, said resin being capable of liberating formaldehyde in amounts in excess of 0.3% based on the weight of the fabric, when stored for 20 hours at 100° F. and at 100% relative humidity which comprises after-treating said resin-treated fabric with between 2% and 15% of a formaldehyde acceptor, said formaldehyde acceptor being a nitrogenous compound capable of reacting with formaldehyde to form a condensation product, said amount of formaldehyde acceptor being based on the weight of the fabric, and thereafter drying the fabric.

4. A process for reducing the amount of formaldehyde liberated from a fabric having a cured formaldehyde liberating resin thereon, said resin being capable of liberating formaldehyde in amounts of between 1 and 3% based on the weight of the fabric, when stored for 20 hours at 100° F. and at 100% relative humidity which comprises after-treating said resin-treated fabric with between about 5% and about 10% of a water-soluble amide formaldehyde acceptor based on the weight of the fabric, said amide being applied as a solution, and thereafter drying the fabric.

5. A process for reducing the amount of formaldehyde liberated from a fabric having a cured formaldehyde liberating resin thereon, said resin being capable of liberating formaldehyde in amounts of between 1 and 3% based on the weight of the fabric, when stored for 20 hours at 100° F. and at 100% relative humidity, which comprises after-treating said resin-treated fabric with between about 5% and about 10% of urea based on the weight of the fabric, said urea being applied as an aqueous solution, and thereafter drying the fabric.

6. A process for reducing the amount of formaldehyde liberated from a fabric having a cured formaldehyde liberating resin thereon, said resin being capable of liberating formaldehyde in amounts of between 1% and 3% based on the weight of the fabric, when stored for 20 hours at 100° F. and 100% relative humidity which comprises after-treating said resin-treated fabric with between about 5 and about 10% of urea based on the weight of the fabric, said urea being applied by spraying an aqueous solution thereof, and thereafter drying the fabric.

7. A process for reducing the amount of formaldehyde liberated from a nylon fabric having a cured formaldehyde liberating resin thereon, said resin being capable of liberating formaldehyde in amounts of between 1% and 3% based on the weight of the fabric, when stored for 20 hours at 100° F. and 100% relative humidity, which comprises spraying said resin-treated nylon fabric with from between about 5 and about 10% of urea, based on

the weight of the fabric, said urea being sprayed as an aqueous solution, and thereafter drying the fabric.

8. A textile fabric treated according to the process of

claim 1.

9. A textile fabric treated according to the process of

claim 6.

10. A nylon textile fabric treated according to the process of claim 7.

References Cited in the file of this patent

UNITED STATES PATENTS

2,267,276 Hager Dec. 23, 1941

FOREIGN PATENTS

312,443 Great Britain May 30, 1929

UNITED STATES PATENT OFFICE  
CERTIFICATE OF CORRECTION

Patent No. 2,833,670

May 6, 1958

Philip B. Roth

It is hereby certified that error appears in the printed specification of the above numbered patent requiring correction and that the said Letters Patent should read as corrected below.

Column 1, line 30, for "alklated" read --alkylated--; column 4, line 44, for "Rochelle netting" read --Rachelle netting--; lines 54 and 55, for "afore-treatment" read --after-treatment--; column 5, line 12, for "Rochelle netting" read --Rachelle netting--.

Signed and sealed this 8th day of July 1958.

(SEAL)

Attest:

KARL H. AXLINE

Attesting Officer

ROBERT C. WATSON  
Commissioner of Patents